

BEST AVAILABLE COPY

W. D. COOLIDGE.

PROCESS OF MAKING COMPOSITE CONDUCTORS.  
APPLICATION FILED SEPT. 23, 1908.

1,010,866.

Patented Dec. 5, 1911.



Witnesses:

George W. Tilden  
J. Ellis Glen.

Inventor:

William D. Coolidge,

by *Albertus Davis*  
Att'y.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## PROCESS OF MAKING COMPOSITE CONDUCTORS.

1,010,866.

Specification of Letters Patent.

Patented Dec. 5, 1911.

Application filed September 23, 1908. Serial No. 454,449.

To all whom it may concern:

Be it known that I, WILLIAM D. COOLIDGE, a citizen of the United States, residing at Schenectady, county of Schenectady, State 5 of New York, have invented certain new and useful Improvements in Processes of Making Composite Conductors, of which the following is a specification.

My present invention has for its object 10 the production of refractory conductors suitable for use in incandescent electric lamps, electric furnaces, and other apparatus where electrical energy is transformed into heat or light.

15 My improved conductor consists in part of refractory metal, such as tungsten, and possesses some of the qualities of a pure tungsten conductor. It has the advantage, however, of a high specific resistance, so 20 high in fact that incandescent lamps can be built for commercial voltages with but a single filament loop. The filament is of such composition that it is strong and comparatively rigid even at the exceedingly high 25 temperatures incident to efficient operation in a lamp.

The details of my improved refractory conductor and of the procedure by which it may be made and used, are set forth in 30 detail in the accompanying description, which should be taken in conjunction with the accompanying drawing. In this description, I have disclosed my invention with special reference to its application to the 35 making of filamentary conductors for incandescent lamps; but the steps disclosed are equally applicable to the making of conductors for other purposes as for use in electric furnaces.

40 As a basis or core for my improved composite conductor, I utilize a thread of thoria or similar refractory oxid. Such threads can be made by mixing pure and finely divided thoria with water and then squirting 45 under pressure through a die. If desired, a small quantity of carbonaceous binder may be mixed with the thoria prior to the squirting operation, though if this is used I prefer to heat the squirted threads with an open 50 flame to burn out the carbon of the binder and leave behind nothing but pure thoria. The next step consists in coating these thoria threads with a ductile metal such as copper. This can be conveniently done in the apparatus shown diagrammatically in the accom- 55

panying drawing. In the drawing is shown an apparatus whereby the thoria threads may be spattered with copper by virtue of the disintegrating action of an electrical discharge passed through a poor vacuum.

60 The apparatus consists of an envelop 1 connected permanently to a vacuum pump and exhausted to a pressure amounting to that of about 1 m. m. of mercury after having been washed out with hydrogen to remove oxidizing gases. At the top of the envelop is supported a copper block 2 provided with electrical connections to render it serviceable as cathode for an electrical discharge. The corresponding anode 3 is 65 passed through the side of the envelop or otherwise suitably arranged. When current is passed from anode to cathode, copper is disintegrated from block 2 and is spattered or deposited on any object placed 70 underneath. This phenomenon is well understood and therefore needs no further explanation. After the thoria threads have been coated with copper as above described, 75 they will conduct current through the copper coating.

80 According to the next step in my process, the copper coated thoria threads are mounted in an envelop and there given a coating of tungsten or molybdenum. This coating 85 can be conveniently effected according to the method disclosed by DeLodyguine in United States Patent No. 575,668; issued January 19, 1897. According to the process 90 there disclosed, the conductors to be coated are heated with current in an atmosphere consisting of a mixture of hydrogen and a volatile compound of a refractory metal, such as the oxychlorid of tungsten. The heated conductor serves to decompose the 95 oxychlorid with depositions of metallic tungsten on the conductor. After a coherent shell of tungsten or similar metal has been produced on the copper-plated thoria threads, the conductor can be heated in hydrogen or in a mixture of hydrogen and nitrogen or in a vacuum to vaporize and distil the copper from the conductor. The copper appears to come out without alloying 100 with the tungsten or in any way influencing its refractory characteristics. Of course, a relatively high temperature is necessary to insure this vaporization of copper but this high temperature is in itself an advantage since it insures partial shrinkage and 105 110

consolidation of the tungsten prior to the liberation of all the copper. After the copper has been removed, the temperature of treatment can be raised by increasing the current and can be continued until the tungsten layer on the thoria thread has been sintered and shrunk into a dense and homogeneous shell.

The composite filament above described has a high specific resistance and, owing to the rigidity of the thoria at high temperatures, is strong and not liable to distortion when used in a lamp. Single loop lamps having commercial voltages are altogether feasible though my invention is not limited in its application to lamps of any particular type or size.

What I claim as new and desire to secure by Letters Patent of the United States, is:

- 20 1. The method which consists in producing a thread of refractory oxid, coating said oxid with a conductor, treating the body so formed to cover it with refractory metal, and subsequently heating to a higher temperature to drive out the conductive layer with which the oxid was initially coated.
- 25 2. The method which consists in shaping threads of refractory material, coating said threads to produce a conductive body, depositing thereon a coating of tungsten and

then driving out of said conductor all components except tungsten and the original refractory material.

3. The method which consists in shaping threads of thoria, coating with a metal, coating again with a more refractory metal, and then heating the conductor so produced to a temperature sufficient to drive out the less refractory metal and leave a composite filament of thoria inclosed in a shell of more refractory metal.

4. The method which consists in shaping a thread of thoria, coating said thread with copper, depositing on said copper a layer of tungsten, and then removing said copper to leave a composite filament of thoria inclosed in a shell of tungsten.

5. The process which consists in producing a thread of refractory material, coating said thread with conductive material, treating the resulting body to cover it with highly refractory material, and heating to a high temperature to drive out said conductive material.

In witness whereof, I have hereunto set my hand this 21st day of September, 1908.

WILLIAM D. COOLIDGE.

Witnesses:

BENJAMIN B. HULL,  
MARGARET E. WOOLLEY.